

Patented Jan. 8, 1946

2,392,611

# UNITED STATES PATENT OFFICE

2,392,611

## DIESEL FUEL

Edwin M. Nygaard, John H. McCracken, and  
Nathan H. Hamilton, Woodbury, N. J., assign-  
ors to Socony-Vacuum Oil Company, Incor-  
porated, a corporation of New York

No Drawing. Application October 20, 1943,  
Serial No. 507,026

13 Claims. (Cl. 44—57)

This invention has to do with fuels for internal combustion engines of the Diesel or compression ignition type and, more particularly, has to do with the improvement of such fuels by the addition thereto of a characterizing ingredient.

In order that a Diesel engine may be operated at maximum efficiency ignition of the fuel should be essentially instantaneous. Delayed ignition or poor coordination between the compression and cylinder conditions is the cause of "knocking" in Diesel operation. As is well known to those familiar with the art, this condition may be remedied by adding small amounts of certain materials or compounds to Diesel or compression ignition fuels. Compounds possessed of such characterizing ability accelerate the ignition of the fuel and thus provide a means whereby the ignition delay period of the fuel is rendered extremely short. In this way, the better grades of Diesel fuels are enhanced and low-grade hydrocarbon mixtures are so improved in ignition quality that they may be used as fuels.

This invention is predicated upon the discovery that compounds represented by the following general formula are effective in improving the ignition quality of a Diesel fuel when used therein in small amounts:



wherein T represents an aromatic group or nucleus, preferably phenyl or naphthyl, which may be unsubstituted or substituted with one or more of such groups as alkyl, aralkyl, aryl, alkaryl, halogen and nitro; R' is a radical selected from the group consisting of alkyl, cycloalkyl, alkaryl, and aralkyl radicals and the same radicals containing a substituent such as halogen or nitro; and R'' is a radical selected from the group consisting of R', halogen and nitro radicals. Typical of the compounds represented by the foregoing general Formula I are the following:

2-(phenylazo)-2-nitropropane,  
2-(2-nitro-4-methyl phenylazo)-2-nitropropane,  
2-( $\alpha$ -naphthylazo)-2-nitropropane,  
1-(phenylazo)-1-chloro-1-nitropropane,  
2-(2-chlorophenylazo)-2-nitropropane,  
2-(3-chlorophenylazo)-2-nitropropane,  
2-(4-chlorophenylazo)-2-nitropropane,  
2-(2,4,6-tribromophenylazo)-2-nitropropane,  
and  
1-(phenylazo)-1-phenyl-1,1-dinitromethane, etc.

Particularly preferred, however, of the compounds so represented are 2-(phenylazo)-2-nitropropane, 2-(3-chlorophenylazo)-2-nitropropane and 2-(4-chlorophenylazo)-2-nitropropane.

It will be apparent that all of the compounds hereinabove represented by general Formula I and contem-

represented above by the general Formula I contain the following characterizing group:



5 wherein the carbon atom, to which an azo group and a nitro group are attached, is also attached to a radical or group such as those represented above by R' and R'', thus being exclusive of attachment of hydrogen. Those related compounds which contain more than one T—N— group attached to a carbon atom which is attached to a nitro group are also contemplated herein as effective Diesel fuel improving agents.

10 It has been found, however, that compounds containing the characterizing group:



15 generally do not improve the ignition qualities of a Diesel fuel. It is most probable that the ineffectiveness of such compounds can be attributed to a rearrangement of the last-mentioned group, the rearrangement taking place in 20 the following manner:



25 30 Illustrative of the compounds of this type (containing characterizing group III) which are ineffective in Diesel fuel are the following:



or



and



or



55

The Diesel fuel improving agents represented

60 hereinabove by general Formula I and contem-

plated herein may be prepared by any of the suitable methods of preparation known in the art, but are preferably prepared by condensing or reacting a salt of a secondary nitroalkane with an unsubstituted aryl, or substituted aryl, diazonium salt, or the corresponding diazonium hydroxide. This preferred method of preparation is described in the following literature articles: Meyer and Ambuhl, Berichte 8, 751-2 (1875), and C. F. Feasley and Ed. W. Degering, J. Org. Chem. 8, 12 (1943); and is illustrated hereinafter by the preparation of several typical compounds represented by general Formula I.

As indicated above, one of the reactants used in the preferred procedure for the preparation of the condensation products contemplated herein is a salt of a secondary nitroalkane. These salts are derivatives of secondary nitroalkanes which may be represented by the following general Formula V:



wherein R' and R'' are as defined hereinabove in connection with general Formula I.

It will be apparent that the salts of the foregoing secondary nitroalkanes may be represented in the following manner:



wherein R' and R'' are as previously defined and M is a metal, and is preferably an alkali metal, such as sodium or potassium. These compounds are well known to those familiar with the art and it is believed that there is no need to refer to methods for their preparation other than those described in the foregoing literature references.

The diazonium compounds which are condensed with the aforesaid nitroalkanes may be represented by the following general formula:



wherein T is as defined above, and X is a diazonium salt group such as one selected from the group consisting of  $-\text{OH}$ ,  $-\text{Cl}$ ,  $-\text{NO}_2$ ,

and  $-\text{OM}$  wherein M is a metal such as sodium or potassium.

From the foregoing, it will be apparent that a salt of a secondary nitroalkane (VI) may be directly reacted with a diazonium compound of the type described above (VII) to form a compound of the type represented above by general Formula I. It will also be apparent that a secondary nitroalkane of the type represented by general Formula V may be used as suggested together with a suitable reagent which will react with said nitroalkane to form the corresponding salt, in the condensation or reaction with said diazonium compound. Among such reagents are the preferred hydroxides, sodium and potassium.

As examples of the compounds contemplated herein as Diesel fuel improving agents, and represented above by general Formula I, are the typical compounds prepared in the following examples:

#### EXAMPLE 1

##### 2-( $\alpha$ -NAPHTHYLATO)-2-NITROPROPANE

$\alpha$ -Naphthyl amine, 1.9 parts by weight, was added to a solution of 12.5 parts by weight of

water and 3.0 parts by weight of concentrated hydrochloric acid. The mixture was diazotized at 0 to 5° C. with 1 part of sodium nitrite dissolved in 4.7 parts of water. To the dark colored solution thus formed was rapidly added 1.5 parts of cold 10% aqueous sodium hydroxide solution and the sodium salt of 2-nitropropane. The last-mentioned compound was prepared by dissolving 1.2 parts of 2-nitropropane in 5.4 parts of 10% aqueous sodium hydroxide. The yellow solid which first formed on the addition of sodium hydroxide solution and the sodium salt of 2-nitropropane changed over to a dark colored tarry like material. The organic layer which formed was separated from the aqueous layer, also formed. The organic product which contained nitrogen was dissolved in Diesel fuel for a test of the cetane number of the resultant oil blend.

#### EXAMPLE 2

##### 2-(4-CHLOROPHENYLATO)-2-NITROPROPANE

To 3.1 parts by weight of para chloroaniline was added a solution of 6.7 parts of concentrated hydrochloric acid in 11.2 parts of water. The mixture was cooled to about 0 to 5° C. A sodium nitrite solution prepared by dissolving 1.7 parts of sodium nitrite in 3.1 parts of water and cooled to 0 to 5° C. was then slowly added to the para chloroaniline hydrochloride in order to diazotize the latter.

The sodium salt of 2-nitropropane was prepared by adding 2.2 parts of 2-nitropropane to an aqueous sodium hydroxide solution obtained by admixing one part of sodium hydroxide and 31.2 parts of water. The solution of the sodium salt was added to a sodium hydroxide solution prepared from 5.2 parts of sodium hydroxide and 62.5 parts of water. Ice, 62.5 parts, was then added to the resulting solution. The diazo mixture prepared above was then added to this ice solution. A yellow precipitate formed immediately. The yellow solid was separated from the mother liquid by filtration and recrystallized from hot ethyl alcohol. The product was a reddish-brown crystalline material melting at 64-67° C.; the literature discloses a melting point of 67.8° C. for 2-(4-chlorophenylazo)-2-nitropropane. The product was analyzed for chlorine and nitrogen, the results being as follows:

|                       | Found | Calculated |
|-----------------------|-------|------------|
| Percent chlorine..... | 14.2  | 15.6       |
| Percent nitrogen..... | 18.2  | 18.5       |

#### EXAMPLE 3

##### 1-(PHENYLATO)-1-CHLORO-1-NITROPROPANE

Aniline (1.3 parts) was dissolved in an aqueous hydrochloric acid solution prepared from the 3 parts of concentrated hydrochloric acid and 13 parts of water. The resulting solution was cooled to about 5° C. by the addition of ice. To the cold solution was added a cold solution of sodium nitrite prepared from 1-part of sodium nitrite and 4.7 parts of water until a positive test for an excess of nitrous acid was indicated by a test with starch-iodide paper. To the diazotized solution was then added 1.5 parts of cold 10 per cent aqueous sodium hydroxide solution, which was followed by an ice cold solution of the sodium salt of 1-chloro-1-nitropropane prepared from 1.7 parts of 1-chloro-1-nitropropane dissolved in 5.4 75 parts of a 10 per cent aqueous sodium hydroxide

solution. The temperature during these operations was maintained at 0 to 5° C. A yellow oil was formed which immediately changed to a dark reddish-brown oil which was separated from the mother liquid, washed with ice cold water and dried by contact with calcium chloride. This product contained nitrogen and chlorine.

The effectiveness of the compounds contemplated herein as Diesel fuel improving agents is illustrated by comparative tests of fuel oil blanks and of fuel oil blends of said fuel oils containing typical compounds or condensation products. The fuel oils used in the test described herein-after are representative Diesel fuels known in the art as catalytically cracked #2 fuel oils and are identified below in Table 1 as Fuel A and Fuel B.

Table 1

| Properties                       | Fuel A | Fuel B |
|----------------------------------|--------|--------|
| Gravity, °A. P. I.               | 23.7   | 31.0   |
| Flash point (Pensky-Martens °F.) | 220    | 187    |
| Aniline point, °F.               | 125    | 119    |
| A. S. T. M. distillation:        |        |        |
| Initial °F.                      | 456    | 421    |
| 10%.                             | 481    | 442    |
| 90%.                             | 589    | 505    |
| End point.                       | 633    | 545    |
| Diesel index.                    | 35.9   | 36.9   |
| Cetane Numer.                    | 33     | 32.4   |

The ignition quality of each of the fuels (A and B) and the fuel blends thereof was determined by a comparison of the same with a standard reference fuel in a converted C. F. R. engine using the ignition delay method. The value shown in this test is expressed as the "centane number" which is the per cent by volume of cetane in  $\alpha$ -methyl naphthalene having the same combustion characteristics as the example under test (reference: Proc. Amer. Soc. Testing Materials, volume 38, I, 392 (1938)).

The results obtained in the foregoing tests with fuel blends containing small amounts of the representative compounds are tabulated in Table 2 below:

Table 2

| Fuel | Improving agent                              | Percent by weight | Cetane number | Increase in cetane No. |
|------|----------------------------------------------|-------------------|---------------|------------------------|
| A    | 2-(phenylazo)-2-nitropropane                 | 1.0               | 37.8          | 4.8                    |
| A    | do                                           | 2.0               | 41.3          | 8.3                    |
| A    | 2-( $\alpha$ -naphthylazo)-2-nitropropane    | 3.5               | 38.4          | 5.4                    |
| A    | 2-(2-chlorophenylazo)-2-nitropropane         | 1.0               | 36.4          | 3.4                    |
| A    | do                                           | 2.0               | 38.1          | 5.1                    |
| A    | 1-phenylazo-1-chloro-1-nitropropane          | 2.0               | 35.6          | 2.6                    |
| B    | 2-(3-chlorophenylazo)-2-nitropropane         | 1.0               | 38.8          | 6.4                    |
| B    | do                                           | 2.0               | 41.9          | 9.5                    |
| B    | 2-(4-chlorophenylazo)-2-nitropropane         | 1.0               | 37.8          | 5.4                    |
| B    | do                                           | 2.0               | 43.0          | 10.6                   |
| B    | 2-(2, 4, 6-tribromophenylazo)-2-nitropropane | 0.5               | 36.6          | 4.2                    |
| B    | do                                           | 1.0               | 37.8          | 5.4                    |

It will be apparent from the foregoing test results that the compounds represented hereinabove by general Formula I are effective in improving the ignition quality of a Diesel fuel. Accordingly, the present invention contemplates a Diesel fuel containing a minor proportion of one or more of the aforesaid compounds for the aforesaid improvement and also contemplates the development of a method for accelerating the ignition of a liquid hydrocarbon fuel in combustion ignition engines, said method being characterized by the

admixture of one or more of said compounds with the fuel prior to its ignition. For the purposes of the present invention, therefore, said compounds may be used in amounts of from about 0.1% to about 5.0%.

It is to be understood that the foregoing examples are illustrative only and not to be construed as in any way limiting this invention. Accordingly, it is to be understood that the term "Diesel fuel" as used herein is inclusive of all types of non-viscous hydrocarbon oils suitable for use in any compression ignition engine.

We claim:

1. An improved Diesel fuel comprising a non-viscous hydrocarbon oil and in admixture therewith a minor proportion, sufficient to improve the ignition quality of the fuel, of a compound containing the characterizing group



wherein T represents an aryl group, and the carbon atom as shown is attached to other than a hydrogen atom.

2. An improved Diesel fuel comprising a non-viscous hydrocarbon oil and in admixture therewith a minor proportion, from about 0.1 per cent to about 5.0 per cent, of a compound containing the characterizing group



wherein T represents an aryl group, and the carbon atom as shown is attached to other than a hydrogen atom.

3. An improved Diesel fuel comprising a non-viscous hydrocarbon oil and in admixture therewith a minor proportion, sufficient to improve the ignition quality of the fuel, of a compound represented by the general formula



wherein T is selected from unsubstituted and substituted aryl groups; R' is a radical selected from the group consisting of alkyl, cycloalkyl, aryl, alkaryl and aralkyl radicals, and said radicals substituted with a substituent selected from the group consisting of halogen and nitro; and R'' is a radical selected from the group consisting of R', halogen and nitro radicals.

4. An improved Diesel fuel comprising a non-viscous hydrocarbon oil and in admixture therewith a minor proportion, from about 0.1 per cent to about 5.0 per cent, of a compound represented by the general formula



wherein T is selected from unsubstituted and substituted aryl groups; R' is a radical selected from the group consisting of alkyl, cycloalkyl, aryl, alkaryl and aralkyl radicals, and said radicals substituted with a substituent selected from the group consisting of halogen and nitro; and R'' is a radical selected from the group consisting of R', halogen and nitro radicals.

5. An improved Diesel fuel comprising a non-viscous hydrocarbon oil and in admixture therewith a minor proportion, sufficient to improve the

ignition quality of the fuel, of a compound represented by the general formula



wherein T represents an aryl group; and R' is a radical selected from the group consisting of alkyl, cycloalkyl, aryl, alkaryl and aralkyl radicals, and said radicals substituted with a substituent selected from the group consisting of halogen and nitro.

6. An improved Diesel fuel comprising a non-viscous hydrocarbon oil and in admixture therewith a minor proportion, sufficient to improve the ignition quality of the fuel, of a compound represented by the general formula



wherein T is selected from unsubstituted and substituted aryl groups; and R' is a radical selected from the group consisting of alkyl, cycloalkyl, aryl, alkaryl and aralkyl radicals, and said radicals substituted with a substituent selected from the group consisting of halogen and nitro.

7. An improved Diesel fuel comprising a non-viscous hydrocarbon oil and in admixture therewith a minor proportion, sufficient to improve the ignition quality of the fuel, of a compound represented by the general formula



wherein T is selected from unsubstituted and substituted aryl groups.

8. An improved Diesel fuel comprising a non-viscous hydrocarbon oil and in admixture therewith a minor proportion, sufficient to improve the ignition quality of the fuel, of 2-(phenyl-azo)-2-nitropropane.

9. An improved Diesel fuel comprising a non-viscous hydrocarbon oil and in admixture therewith a minor proportion, sufficient to improve the ignition quality of the fuel, of 2-(3-chloro-phenylazo)-2-nitropropane.

10. An improved Diesel fuel comprising a non-viscous hydrocarbon oil and in admixture therewith a minor proportion, sufficient to improve the

ignition quality of the fuel, of 2-(4-chloro-phenylazo)-2-nitropropane.

11. The method of accelerating the ignition quality of a liquid hydrocarbon fuel in an engine where the fuel is injected into the engine cylinder and ignites spontaneously therein, which comprises admixing with the fuel prior to its ignition in the cylinder, a minor proportion of a compound containing the characterizing group



wherein T represents an aryl group, and the carbon atom as shown is attached to other than a hydrogen atom.

12. The method of accelerating the ignition quality of a liquid hydrocarbon fuel in an engine where the fuel is injected into the engine cylinder and ignites spontaneously therein, which comprises admixing with the fuel prior to its ignition in the cylinder, a minor proportion of a compound represented by the general formula



wherein T is selected from unsubstituted and substituted aryl groups; R' is a radical selected from the group consisting of alkyl, cycloalkyl, aryl, alkaryl and aralkyl radicals, and said radicals substituted with a substituent selected from the group consisting of halogen and nitro; and R'' is a radical selected from the group consisting of R', halogen and nitro radicals.

13. The method of accelerating the ignition quality of a liquid hydrocarbon fuel in an engine where the fuel is injected into the engine cylinder and ignites spontaneously therein, which comprises admixing with the fuel prior to its ignition in the cylinder, a minor proportion of a compound represented by the general formula



wherein T is selected from unsubstituted and substituted aryl groups.

EDWIN M. NYGAARD.  
JOHN H. McCACKEN.  
NATHAN H. HAMILTON.